

May 24, 1932.

G. B. STRYKER, JR.

1,860,060

METHOD OF MAKING SHINGLES

Filed July 31, 1928

Fig. 7.



Fig. 5.



Fig. 2.



Fig. 1.



Fig. 8.



INVENTOR.

George B. Stryker  
H. H. Payne

ATTORNEY.

## UNITED STATES PATENT OFFICE

GEORGE B. STRYKER, JR., OF MEMPHIS, TENNESSEE, ASSIGNOR TO THE WEATHERPROOF PRODUCTS COMPANY, OF MEMPHIS, TENNESSEE, A CORPORATION OF TENNESSEE

## METHOD OF MAKING SHINGLES

Application filed July 31, 1928. Serial No. 296,604.

The present invention has for its object a method of manufacturing articles such as are described in my co-pending application entitled "Shingle construction and composition", Serial No. 296,603, filed simultaneously herewith.

It relates to a composite shingle comprising two separate and distinct elements which are so intimately joined together that they 10 form an inseparable unit. As the physical properties of one element differ considerably from the properties of the other the composition of the "mix" for each is also different. The base or core element is soft and porous, 15 like a felt pad and is a good heat and cold insulator. The other element composed principally of mineral ingredients possesses a hard surface and has accordingly good wearing properties, is rain- and hail-proof and a 20 non-conductor of electricity.

In the accompanying drawings is illustrated a composite shingle made in accordance with the present invention, and

Figure 1 is a plan view of the base element 25 of the shingle; and

Figure 2 is an end view of Figure 1;

Figure 3 an under plan view of the top or cover element of the shingle; and,

Figure 4 an end view of Figure 3;

Figure 5 is a bottom plan view of the assembled shingle;

Figure 6 a transverse section along line 6—6 of Figure 5;

Figure 7 a longitudinal section along line 35 7—7 of Figure 5;

Figure 8 is a fragmentary plan view of a roof laid with these shingles; and

Figure 9 a fragmentary section along line 9—9 of Figure 8.

Reference numeral 10 represents the base or core element and numeral 11 the top or cover element. By means of the marginal flanges 12 the top element 11 grips tightly the edges of the base element 10 on three sides. To insure still further hold between the two elements, the side edges of the base element are preferably provided with indentations or notches as at 13, while the flanges of the top element have corresponding sharp projections 14 engaging said notches.

The lower end of the base element is slightly tapered as from 15 to 16 for the purpose of increasing the flange thickness of the top element, thereby giving greater strength and also preventing water from reaching the base element. For the same reason the flanges 12 are made slightly higher, as at 18, than the thickness of the pad or base element, which preferably has uniform thickness. In this manner when the shingle is laid the bottom surface of the pad or base element will be raised above the supporting structure.

As best seen in Figure 5 of the drawings the finished shingle is preferably rectangular, that is to say, the top element has parallel side edges which merge into the edges of the upper portion 17 of the base element, while the remainder of the latter has the same contour as the inner side of the flanges 12.

The body portion 19 of the top or cover element 11 tapers slightly from one end to the other, being thickest at the lower end as at 18 where it is of the same or greater thickness than the base element, while running out to a knife edge a little short of the top edge of the base element 10 or about midway between said edge and the notches 14. At 22 are shown nail holes in the top element for securing the shingles in position.

In Figures 8 and 9 is illustrated the preferable manner of laying the shingles. A tier of units A is first nailed fast as at 22 and positioned with the butt ends 23 lowermost, in a straight line in the usual manner. The next tier B is then placed on top of the first with its line of butt ends 23 about six inches from the first butt end line or about even with points 15 of Figure 1. This then provides the exposed or "weather" portion of units A. At the same time the side edges of the units in tier B are displaced about one-third of the width of the shingle from the side edges of tier A as seen in Figure 8. This gives a staggered line of exposed side edges. Similarly the third and fourth tiers C of shingle units are laid and nailed fast to produce the assembled effect indicated.

The preferred size of a shingle unit is six

55

60

65

70

75

80

85

90

95

100

inches by fourteen inches (6" x 14") distributed as follows: 2" from the upper edge to the notch 13; 6" between said notch and the point 15; and 6" below the latter. In this manner there will always be three thicknesses of shingle near its upper and lower edge of 2" length, while 10" will have double thickness and only 6" will be exposed.

The product may have many other applications than the one shown on the drawings of which a few may here be enumerated, namely as wallboards, fillers, electric insulating material, weather sidings, linings, surfacing and exterior veneering of building walls.

The production of the base or core element will first be treated. This element is made in a similar manner as paper or cardboard so as to form large sheets which are subsequently cut up into pads of suitable size and contour and preferably of uniform thickness.

The preferred method of manufacturing this base element is here described but it is evident that many modifications may be made and particularly as regards the ingredients selected, the latter depending mainly on the locality where the articles are manufactured, so that in the south, where cotton stalks are abundant these would form the basic ingredients; while in other places, where corn stalks, wood shavings or the like abound, they would form the base as being the cheapest and easiest to obtain.

The ingredients for the mix are principally fibre, as from cotton stalks and waste paper, preferably old newspapers. Of these ingredients approximately 75% in weight of fibre is taken with 25% of paper waste, finely comminuted and placed in a mechanical mixer together with sufficient water to produce a flowing substance or mix of creamy consistency. The water should be heated sufficiently, say to 250 or 300 degrees Fahrenheit, in order to act on the binder contained in the waste paper. In case more binder is found necessary, finely comminuted rosin may be dissolved in the hot water before added to the other ingredients in the mechanical mixer. When rosin is used the weight proportions would be approximately 67 to 73% cotton stalk or other vegetable fibre, 25% waste paper and 8 to 2% rosin.

The creamy mix is then pumped from the mechanical mixer and passed through rolls, which should be heated and on to an endless belt, as in paper making, forming long sheets which are subsequently cut or in any suitable manner divided and shaped into pads of required size and form.

The top or cover element is next produced in the following preferred manner but it is also here evident that many modifications may be made particularly in the selection of the ingredients.

The ingredients are fibre, clay, lime, and

cement, to which may be added any coloring material desired.

First, the fibre is finely comminuted. For this ingredient, any kind of vegetable fibre may be used and in particular cotton stalks, 70 but even asbestos fibre may be used.

Next clay, so-called "ball clay" preferably, is similarly brought into pulverized state.

Hydrated lime and Portland cement are then treated in the same manner to be finely 75 comminuted.

These ingredients are thereupon put into a mechanical mixer in the approximate weight proportions of 3, 6, 2 and 18, respectively; or for a single shingle, for instance, 80 1.5 ounces of the fibre, 3 ounces of the ball clay, 1 ounce of the hydrated lime and 9 ounces of Portland cement, all finely comminuted, are stirred up in the mixer together with water until a fine, plastic mix is obtained. In case coloring is desired, any desired coloring material is added to the mix 85 while being stirred.

This plastic mix is now ready to be cast and a suitable mold of the size and shape of the article to be made is used. For the composite shingle shown in the drawings the mold has a rectangular recess of the length, width and depth of the shingle, as seen in Figures 5, 6 and 7, and its bottom is slanting 95 towards one end. A filler piece of wood or felt is first placed on the bottom of the mold recess and this filler piece is cut to the size and shape of the base element as seen in Figure 1 and temporarily or permanently secured in the mold bottom. Its thickness is equal to the difference between the height of the flange 12 of the top element 11 and the thickness of the pad or base element 10, see 100 Figure 7.

The base element 10 which has previously been dried and completely finished is next placed on top of the filler piece. The plastic mix is now poured into the mold and pressure applied in order to squeeze the mix 105 tightly around three edges of the pad or base element and into the notches at 13 thereof. The pressure is continued until the mass becomes firm and hard, when the body portion 19 of the top element will cover the top side of the base element 10 tapering from the butt end 23 to nothing short of the other end of the pad as seen in the figures.

As soon as the plastic mix is perfectly dried 110 out the now finished composite shingle is removed from the mold ready for use. The two elements adhere very firmly to each other on account of the shape of the elements and their treatment.

The required pressure during the casting 115 may be obtained either from a mechanical, air or hydraulic press.

It is to be understood that the invention as 120 here disclosed is not limited to the details of composition and steps in the process but 125 130

that these may be varied widely without departing from the spirit of the invention as defined by the claims.

What I claim as new is:

1. A method of manufacturing a composite structural unit comprising a body portion and a cover portion, which consists in thoroughly mixing finely comminuted fibre, paper, and a suitable binder in the presence of hot water until the mass has a creamy consistency, passing the mass through heated pressing rollers to form a sheet, cutting the resultant sheet into suitable shapes for said body portions; mixing finely comminuted fibre, clay, lime and cement into a plastic mass, placing said body portion in a mould and then pouring thereon said plastic mass and applying pressure thereto whereby said mass will tightly bind against the body portion and produce the structural unit, substantially as set forth.

2. A method of manufacturing a composite structural unit comprising a body portion and a cover portion, which consists in thoroughly mixing, by weight, finely comminuted fibre 67 to 73%, waste paper 25%, and rosin binder 3 to 8%, in the presence of water heated to 250° or 300° F. until the mass has a creamy consistency, passing the mass through heated pressing rollers to form a sheet, cutting the resultant sheet into suitable shapes for said body portions; next mixing finely comminuted fibre, clay, lime and cement into a plastic mass, placing said body portion in a mould and then pouring thereon said plastic mass and applying pressure thereto whereby said mass will tightly bind against the body portion and produce the structural unit, substantially as set forth.

3. In witness whereof, I have hereunto set my hand at Washington, District of Columbia, this twenty-seventh day of July, A. D. nineteen hundred and twenty-eight.

GEORGE B. STRYKER, JR.

45

50

55

60

35